

[54] PROCESS FOR THE PRODUCTION OF HIGH STRENGTH YARNS BY SPIN-STRETCHING AND YARNS PRODUCED BY THE PROCESS, ESPECIALLY FROM POLYAMIDE-6 AND POLYESTER FILAMENTS

[75] Inventors: Günter Koschinek, Dietzenbach; Dietmar Wandel, Hanau, both of Fed. Rep. of Germany

[73] Assignee: Davy McKee Aktiengesellschaft, Fed. Rep. of Germany

[21] Appl. No.: 281,595

[22] Filed: Jul. 9, 1981

[30] Foreign Application Priority Data

Jul. 12, 1980 [DE] Fed. Rep. of Germany ..... 3026451

[51] Int. Cl.<sup>3</sup> ..... D01D 5/16  
 [52] U.S. Cl. ..... 264/210.3; 264/210.8;  
 ..... 264/342 RE

[58] Field of Search ..... 264/195 F, 342 RE, 210.3,  
 ..... 264/210.8

[56]

References Cited

U.S. PATENT DOCUMENTS

|           |         |                     |           |
|-----------|---------|---------------------|-----------|
| 3,715,421 | 2/1973  | Martin et al. ....  | 264/210.8 |
| 4,003,974 | 1/1977  | Chantry et al. .... | 264/210.8 |
| 4,070,432 | 1/1978  | Tamaddon ....       | 264/210.3 |
| 4,228,120 | 10/1980 | Bromley et al. .... | 264/176 F |
| 4,229,500 | 10/1980 | Adachi et al. ....  | 264/210.8 |
| 4,237,187 | 12/1980 | Raybon et al. ....  | 264/176 F |
| 4,251,481 | 2/1981  | Hamlyn ....         | 264/210.3 |

FOREIGN PATENT DOCUMENTS

50-25819 3/1975 Japan ..... 264/210.8

Primary Examiner—Jay H. Woo

Attorney, Agent, or Firm—Allegretti, Newitt, Witcoff & McAndrews, Ltd.

[57]

ABSTRACT

An improved process for the spin-drawing of high-tensile, technical-grade yarns is disclosed. The process produces yarns of high industrial quality having a low break elongation and low reference elongation, or a low heat shrinkage and low reference elongation. The process is especially suitable for yarns of polyamide and polyester.

12 Claims, 3 Drawing Figures



FIG. 1





FIG. 2



FIG. 3

PROCESS FOR THE PRODUCTION OF HIGH STRENGTH YARNS BY SPIN-STRETCHING AND YARNS PRODUCED BY THE PROCESS, ESPECIALLY FROM POLYAMIDE-6 AND POLYESTER FILAMENTS

BACKGROUND OF THE INVENTION

The invention relates to a process for the production of high-tenacity technical-grade yarns, particularly of polyamide and polyester, having a low reference elongation, by spin-drawing, in which the filaments extruded from a spinneret are cooled in a cooling zone by being exposed to a stream of air, are passed over a preparation device, and then passed directly over several sets of rolls to be drawn, in at least one draw field, between at least two of the sets of rolls. The filaments are subjected to a temperature of at least 160° C. in at least one set of rolls and, finally, are passed over a set of let down rolls prior to being wound up at a speed of at least 2,200 meters/min.

In order to use the yarns for straps, belts and layer webs for textile fabrics, the heat shrinkage of the yarns should be low and, at the same time, the lowest possible reference elongation should be sought.

Feed yarns made from polyamide or polyester will undergo a change in textural condition during the various process stages. In the article, "Spinning Process and Crystal Structure of Perlon," *Angewandte Chemie*, Vol. 74, 1962, No. 13, p. 566, it is noted that a yarn drawn directly during the spinning operation passes through crystallization stages that are different from those of a yarn made on a drawing machine from staple stock.

Furthermore, at higher production speeds, a uniform temperature transfer to the yarn becomes more difficult. Higher speeds also translate into shorter contact times between the yarn and the heating systems, so that the heating of the yarn to predetermined temperatures becomes more of a problem. However, it is the temperature and structural properties which largely determine the attainable qualities of textile yarn.

The technical and economical value of the spin-draw process, however, can be rated as positive only if, at the same time, the textile yarn qualities are not impaired and even improved.

From German published patent application No. 1,435,467, a process for spin-drawing of polyester (PES) at speeds of 1000 to 4000 m/min. is known. The process disclosed therein utilizes a temperature treatment of the filaments at predetermined residence times prior to the drawing operation. However, no process parameters for drawing and thermal stabilizing, such as temperature control and yarn tensions, are disclosed. In applying the teachings of this reference, low reference elongation values were generally obtained in combination with high tenacities and low elongation or low shrinkage values.

U.S. Pat. No. 3,452,131 and German published patent application No. 1,912,299 disclose processes for the spin-drawing of polyamide filaments in which additional draw means are employed. In the case of a steam jet, there is a danger of simultaneous wetting or moistening because of the low yarn temperature, a fact which is well known, and which has a substantial influence on the glass transition point. At high speeds, i.e., short residence times, this expedient may lead to complications in the drawing process. The use of a stationary

draw pin is known from conventional methods, but is recommended only for moderate speeds. At high speed production, the friction is too strong causing the increase in temperature of the pin to be uncontrollable.

5 Both of these references fail to make any recommendations as to how low reference elongations might be attained.

If, in spin-drawing, the cooled filaments are drawn at high speeds on stationary draw means, and if, for the purpose of increasing productivity, more than one strand of filaments is processed at one station, there is danger of non-uniform draw action, particularly among the yarns at different stations.

10 U.S. Pat. No. 3,790,995 discloses a process for spin-drawing of polyester at speeds of at least 1800 m/min, in which the feed and draw rolls are provided with a surface roughness to allow slippage of the continuous filaments over a number of wraps on the rolls. Such filament slipping leads to a high degree of friction at high production speeds, and the frictional heat generated causes an uncontrollable increase in temperature of the rolls. No teaching can be derived from the given parameters of this reference as to how to achieve a low reference elongation.

15 U.S. Pat. No. 4,003,974 discloses a process for spin-drawing of polyester, in which the filaments are thermally stabilized or "set" at 225°-250° C., and are allowed to relax at a tension of 0.09-0.15 g/den, with a speed given, by way of example, as 1.829 m/min. It does not teach an operation at higher speeds. The given temperatures could not be further increased because temperatures in the range of the polymer melting point cause the filaments to stick to the rolls. An increase in

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905

being the temperature of the glass transition point, and the filaments are drawn without the use of additional stationary draw means;

(b) The sets of rolls following the minimum of one draw zone have a temperature in excess of 110° C., and the tension of the yarn after leaving these roll systems is not less than 0.2 g/dtex;

(c) The residence time of the yarn in the let down roll system is selected to be at least 0.2 sec.;

(d) The windup speed of the yarn does not decrease by more than 2.5% from the peripheral speed of the let down roll system; and

(e) The temperature of the system of let down rolls is adjusted to a value of less than or equal to 110° C.

The yarn packages thus produced can be used directly on a thread machine without requiring any additional process steps. Plying and twisting of the yarn will produce cord for further processing in textile manufacture.

By combining the two operational steps of spinning and drawing, the coupled spin-drawing process saves a separate operation, and, by employing high windup speeds, it becomes extremely economical.

The drawn feed yarns meet high quality requirements because of their predictable technical performance in the manufacture of woven and other textiles.

Feed yarn used in the manufacture of tire cord requires, in addition to other properties, first and foremost, a high degree of tenacity, low break elongation and low reference elongation. These conditions are also met by the product of the present invention.

The characteristic features of the invention define for each process step a specific treatment of the yarn, as determined by yarn temperatures, yarn residence times and yarn tensions, so that a combination of the inventive features will yield the desired yarn characteristics. The heating of the filament yarn on the rotating rolls is sufficient to permit a precise adjustment of the temperature necessary for the drawing operation and the thermal treatment. The upper limit of temperatures of 40 greater than or equal to 160° C. employed in the thermal setting step of the yarn is defined by the instant the yarn adheres to the rolls, i.e., when the temperature range of the polymer melting point has been reached. Hence, the maximum possible temperature is higher for polyester than it is for polyamide-6. In conventional processes, the yarn then may pass into a low tension zone of less than or equal to 0.2 g/dtex thereby causing a considerable shrinkage of the yarn, depending on the yarn temperature. Such relaxation of the yarn is in part desired because the tendency of the finished yarn to shrink in hot air is thereby lessened, i.e., a yarn is obtained having a low dry heat shrinkage value. In conventional processes, relaxation tensions of less than or equal to 0.15 g/den are employed to obtain dry heat shrinkage values (at 160° C.) of less than or equal to 4%. This, however, is accompanied by a strong increase in reference elongation, which is undesirable for technical-grade material. Consequently, it is necessary to limit the relaxation tension to greater than or equal to 0.2 g/dtex to obtain a low reference elongation, along with low dry heat shrinkage.

To eliminate relaxation to a large extent, tensions of greater than or equal to 1.0 g/dtex are employed, so that yarns having a low break elongation and low reference elongation are obtained. If the let-down roll is heated for the thermal stabilization step of the yarn, the heated yarn, upon leaving the let-down roll, directly enters a

region of low tension, which is usually adjusted at less than 0.2 g/dtex prior to the windup operation and a stable build-up of the yarn package. However, since the yarn temperature is much higher than 110° C., the reference elongation will be strongly increased, as in Example 6 herein.

Even if the let-down roll is not heated, the yarn heated on the roll effecting the thermal stabilization transfers considerable quantities of heat to the let down roll. At medium speeds of less than 2,200 m/min and thermal setting temperatures of 190°-250° C., conventional let down rolls will heat up to temperatures of 55°-85° C. Increasing the speed may cause the roll temperature to rise up to 115° C. The yarn leaving the roll then has a relatively high temperature and experiences a strong and undesirable shrinkage. If, however, the let rolls are cooled, the yarn temperature will decrease accordingly and the tendency of the yarn to shrink is curtailed to a large extent.

While the heating of the yarn by contact with rolls at high production speeds is difficult, the cooling carried out under the conditions according to the present invention has produced a positive effect. The preferred let down roll system consists of at least one driven roll and may include additional rolls, not driven and freely mounted, and a stretch or zone of free space between the rotating aggregates. The flow of air, especially in the zone of free space, produces a special cooling effect if the total residence time is at least 0.2 sec.

The speed ratio between the let-down roll and the windup device directly determines the shrinkage of the yarn and, in combination with the associated yarn tension, also the shrinkage tendency of the yarn on the bobbin. For these reasons, the speed ratio must not exceed the specified limit. Under conventional conditions, the ratio is in excess of 2.5% with a usual windup tension of less than 0.2 g/dtex. However, only with yarn cooled as proposed by the present invention can low ratios be realized. Such yarns then have a lower shrinkage propensity and, hence, a lower value of the reference elongation.

The process of the invention may be carried further to best advantage through the following steps:

(1) the filaments extruded from the spinneret are passed through a heat zone before they enter the cooling zone;

(2) for the preparation of the filaments, an oil having less than 5% by weight of water, particularly a water-deficient oil, is applied to the filaments in the absence of heat;

(3) the let down roll system is unheated and is provided with cooling means enabling a surface temperature of less than or equal to 25° C.;

(4) in the proximity of the set of let down rolls, a cooling zone is provided having a temperature of less than or equal to 25° C. to enable a heat exchange with the yarn;

(5) the residence time of the yarn in the cooling zone is adjusted to be at least 0.4 sec;

(6) the set of let-down rolls is positioned in a closed environment, the temperature of which is maintained by forced cooling at or below 45° C.;

(7) the tension of the withdrawn yarn is not less than 0.5 g/dtex;

(8) the set of rolls positioned downstream of the drawing zone has a temperature of at least 160° C. and the yarn tension of the withdrawn yarn is not less than 1.0 g/dtex; and

(9) the yarn is passed through a whirling unit prior to being wound up in order to improve the closing off of the yarn end.

The process of the present invention will be described in further detail with reference to a preferred embodiment illustrated in FIGS. 1-3 and several process examples. The characteristics of all examples are summarized in the table at the end of the description.

#### BRIEF DESCRIPTION OF THE DRAWINGS

FIG. 1 is a diagrammatic illustration of an apparatus for use with a preferred embodiment of the process according to the present invention.

FIG. 2 is a graph showing the relation between reference elongation (ordinate) and heat shrinkage (abscissa).

FIG. 3 is a graph showing the relation between reference elongation (ordinate) and break elongation (abscissa).

#### DETAILED DESCRIPTION OF THE PREFERRED EMBODIMENTS

Referring to FIG. 1, a spinneret 1 has a multiplicity of orifices or holes in a spinning block 2. Filaments 3, which subsequently form continuous filament strands or yarn are extruded from the spinneret 1 and are passed through a heater 4 enclosing a heating zone 4a. The filaments 3 then pass through a blow duct 5, enclosing a cooling zone 5a, in which the filaments are cooled by an air current blowing in the direction of the arrows 6.

Below the blow duct 5, a preparation system 7 is arranged by which a finish or preparation is applied to the filaments. Following is a first set of rolls 8 ("first duo"), which may be designated a feed roll system and which is heated to a temperature of  $T_G - 20^\circ \text{ C.}$  to  $T_G + 65^\circ \text{ C.}$  based on the glass transition point. The continuous filaments 3 are passed over this roll system 8.

The first roll system 8 is followed by a second roll system 9 ("second duo"), which may be termed a draw roll system, and over which the filaments 3 also are passed. Located between the two roll systems 8 and 9 is a draw zone "V." The roll system 9 consists of rolls which have a temperature of more than  $110^\circ \text{ C.}$  and the strands of filaments 3 leaving this roll system have a yarn tension of at least 0.2 g/dtex. In the case where only a single roll system 9 is provided, subsequent to the draw zone, as shown in FIG. 1, this roll system is additionally and simultaneously adapted to fulfill the condition that the respective rolls have a temperature of at least  $160^\circ \text{ C.}$

Following the roll system 9 is a let-down roll system 10 ("third duo") which, like the roll systems 8 and 9, is in the form of a "duo," i.e., it consists of two rolls 10a and 10b. In the region of the roll system 10, a cooling zone 11 is formed which is located inside a roll box or casing 12 enclosing the rolls 10a and 10b. The arrangement of the rolls 10a and 10b is such that the residence time of the strands of filaments 3 in the let-down roll system 10 and the cooling zone 11, respectively, is at least 0.2 sec. The temperature of the let-down roll system 10 is no greater than  $110^\circ \text{ C.}$

Finally, a windup unit 13 is provided for the takeup of the yarn 3. The peripheral speed of the windup 13, at the point of first contact with the yarn, decreases by no more than 2.5% from the peripheral speed of the let-down roll system 10.

The present invention can be better understood with reference to the following examples. Characteristic values used in the following examples are based on the following measuring procedures: Tenacity and break elongation were measured on conventional tensile testing equipment. The reference elongation was determined from the load/extension diagram of the yarn. The reference elongation is defined as the elongation of the yarn at a force of 4.85 g/dtex.

#### EXAMPLE 1

Polyamide-6 having a relative viscosity  $n_{rel}$  of 3.3 was melted at  $293^\circ \text{ C.}$  and was passed at a rate of 247 g/min through two spinneret plates each having 140 holes, each hole having a diameter of 0.4 mm.

The extruded filaments were passed through a 600 mm long heater having a wall temperature of  $300^\circ \text{ C.}$ , and were subsequently passed through a 1100 mm long blow duct in which they were cooled by a transversely directed air current blowing at a speed of 0.8 m/sec.

Thereafter, a 99% preparation was applied to the filaments by means of cold rolls, so that the oil film on the finished feed yarn was 1.1%.

The continuous filaments were then drawn between two sets of rolls (duos) at a temperature of  $90^\circ \text{ C.}$  and a draw ratio of 1:5.1, were thermally stabilized on the second duo at a temperature of  $195^\circ \text{ C.}$ , were passed over the unheated let-down roll system at a temperature of  $45^\circ \text{ C.}$  and a speed of 2,805 m/min, and then through a cooling zone having an ambient temperature of  $40^\circ \text{ C.}$ , and were finally wound up at a speed of 2,740 m/min.

Disregarding the permissible amount of shrinkage between duo 2 and duo 3, the thermal setting tension was 2.1 g/dtex, the windup tension was 150 g, and the denier of the wound up yarn was 940/140 dtex. The residence time of the yarn in the let-down or relaxation roll system was 0.72 sec.

No disturbances occurred in the drawing operation. The yarn characteristics are reported in Table 1. A high tenacity was obtained as well as a low break elongation and a low reference elongation.

#### EXAMPLE 2

Polyamide-6 filaments were extruded and spin-drawn under the same conditions as in Example 1, except that the temperature of the let-down roll system was adjusted to  $60^\circ \text{ C.}$  and the cooling zone temperature was  $32^\circ \text{ C.}$  The values reported in Table 1 show a further improvement in the reference elongation. The tenacity was somewhat lower and the break elongation was slightly higher than in Example 1.

#### EXAMPLE 3

Polyamide-6 filaments were extruded and spin-drawn under the same conditions as in Example 2, except that two pairs of rolls operating at the same speed were used as the let-down roll system. The pair of rolls, first engaged by the filaments, had a temperature of  $60^\circ \text{ C.}$ , the second pair of rolls had a temperature of  $34^\circ \text{ C.}$ , and the cooling zone had a temperature of  $23^\circ \text{ C.}$  The residence time of the yarn in this system was 2.7 sec. There were no difficulties during the drawing operation. The yarn showed a low break elongation and a low reference elongation coupled with a high tenacity.

**EXAMPLE 4**

### (Comparison Example)

Polyamide-6 filaments were extruded and prepared under the same conditions as in Example 1. The filaments were drawn between two sets of rolls (duos) at a temperature of 90° C. and a draw ratio of 1:5.1. They were allowed to thermally set on the second duo at a temperature of 195° C., were passed over unheated let down rolls operating at a speed of 2,805 m/min, and finally were wound up at a speed of 2,675 m/min.

The temperature of the let-down rolls adjusted itself after a short initial period of a few seconds to a surface temperature of 112° C. The residence time of the yarn on these rolls was 0.15 sec. Disregarding the permissible amount of shrinkage occurring between duo 2 and duo 3, the setting tension was 2.1 g/dtex. The windup tension was 150 g. The finished yarn thus produced exhibited a strong shrinkage propensity during the windup which had an adverse effect on the buildup of the yarn package. The yarn showed a low tenacity and a higher break elongation than in Example 1. The reference elongation was substantially higher than in the previous examples.

### EXAMPLE 5

Polyamide-6 having a relative viscosity  $n_{rel}$  of 2.8 was melted at 284° C. and was extruded at a rate of 247 g/min through a spinneret plate with 140 holes, each hole having a diameter of 0.4 mm. The extruded filaments were passed through a 1700 mm long blow duct in which they were cooled by a transversely directed current of air blowing at a speed of 0.6 m/sec. Thereafter, a 99% preparation was applied to the filaments by cold rolls, so that the oil film on the finished yarn was 0.8%.

The filaments were then drawn between two sets of rolls (duos) at a temperature of 90° C. and a draw ratio of 1:5.1. On the second duo, the continuous filament strands were allowed to thermally set, were passed over the unheated let-down roll system operating at a speed of 2,805 m/min, and were finally wound up at a speed of 2,790 m/min. The let-down rolls were water cooled and maintained at a temperature of 23° C. The cooling zone had an ambient temperature of 20° C. The residence time in the let-down roll system was 1.6 sec. At a relaxation tension of 0.22 g/dtex between duo 2 and duo 3 and a windup tension of 150 g, a denier of 940/140 dtex was obtained.

The yarn thus produced had a dry heat shrinkage of 3.5% and a reference elongation of 8.5%. The break elongation was about 19.8%.

### EXAMPLE 6

### (Comparison Example)

Polyamide-6 filaments were extruded and spin-drawn under the same conditions as in Example 5, except that the let-down roll was adjusted to a temperature of 195° C., the yarn residence time was 0.15 sec., and the 60 windup speed was 2,635 m/min.

While the yarn thus obtained showed a dry heat shrinkage of 3.7%, which is comparable to the result of Example 5, it had a substantially higher reference elongation of 12%. The break elongation of 24% was clearly higher.

### EXAMPLE 7

Polyester having a relative viscosity  $\eta_{intr}$  of 0.68 was melted at 305° C. and was extruded at a rate of 307 g/min from two spinneret plates, each having 192 holes, each hole having a diameter of 0.4 mm. The extruded filaments were passed through a 1700 mm long blow duct in which they were cooled by a transversely directed stream of air flowing at a speed of 0.6 m/sec. Thereafter, a 99% preparation was applied to the filaments by cold rolls, so that the oil film of the finished yarn was 0.7%.

The filaments were then drawn between two sets of rolls (duos) at a temperature of 115° C. and a draw ratio of 1:6.1. On the second duo, the filaments were allowed to thermally set at a temperature of 220° C., were then passed over the unheated let-down roll system at a temperature of 45° C. and a speed of 3,050 m/min, and through the cooling zone at a temperature of 38° C., and were finally wound up at a speed of 2,990 m/min.

With a permissible amount of shrinkage between duo 2 and the let-down roll system, with a relaxation tension of 0.2 g/dtex and a windup tension of 170 g, a yarn of 1100/192 dtex denier was obtained. The residence time 30 of the yarn in the let-down roll system was 0.22 sec. No disturbances occurred during the drawing operation. The dry heat shrinkage was 3.5%, the reference elongation was 7.6%, and the break elongation was about 13.5%.

35 In a subsequent run, the permissible amount of shrinkage between duo 2 and the let-down roll system was varied, all other conditions remaining equal. The setting tension increased to 1.2 g/dtex.

40 By this modification of the process, it is possible to obtain yarns having the desired reference elongation, up to about 5%, and a low break elongation, as is shown in FIG. 2, in which the abscissa represents the dry heat shrinkage and the ordinate represents the reference elongation, each in percentage. It will be noted, however, that, with low reference elongations, the dry heat shrinkage increases. In FIG. 3, the abscissa shows the break elongation and the ordinate shows the reference elongation, each in percentage. The graphs illustrate Example 7, i.e., they are representative of polyester.

### EXAMPLE 8

### (Comparison Example)

55 Polyester filaments were extruded and spin-drawn under the same conditions as in Example 7, except that the unheated let-down roll system, after an initial period of a few seconds, heated itself up to a temperature of 115° C.

With about the same dry heat shrinkage value as in Example 7, a substantially higher reference elongation of 9.9% was obtained. The tenacity value was clearly lower.

TABLE 1

TABLE 1-continued

| Example No.<br>Invention/Comparison                    | 1<br>Invention | 2<br>Invention | 3<br>Invention | 4<br>Comparison | 5<br>Invention | 6<br>Comparison | 7<br>Invention | 8<br>Comparison |
|--------------------------------------------------------|----------------|----------------|----------------|-----------------|----------------|-----------------|----------------|-----------------|
| 1st down rolls 10                                      | 2,805          | 2,805          | 2,805          | 2,805           | 2,805          | 2,805           | 3,050          | 3,050           |
| windup unit 13                                         | 2,740          | 2,740          | 2,740          | 2,675           | 2,790          | 2,635           | 2,990          | 2,925           |
| Draw ratio 1:                                          | 5.1            | 5.1            | 5.1            | 5.1             | 5.1            | 5.1             | 6.1            | 6.1             |
| Admissible shrinkage %                                 | 0              | 0              | 0              | 0               | 6              | 6               | 5              | 5               |
| Temp. roll system 8 °C.                                | 90             | 90             | 90             | 90              | 90             | 90              | 115            | 115             |
| roll system 9 °C.                                      | 195            | 195            | 195            | 195             | 195            | 195             | 220            | 220             |
| let-down roll 10 °C.                                   | 45             | 60             | 60/34          | 112             | 23             | 195             | 45             | 115             |
| roll box °C.                                           | 40             | 32             | 23             | 23              | 20             | 20              | 38             | 38              |
| Setting tension g/dtex                                 | 2.1            | 2.1            | 2.1            | 2.1             | 0.22           | 0.22            | 0.2            | 0.2             |
| Windup tension g                                       | 150            | 150            | 150            | 150             | 150            | 150             | 170            | 170             |
| Residence time of the yarn in the let down system sec. | 0.72           | 0.72           | 2.7            | 0.15            | 1.6            | 0.15            | 0.22           | 0.22            |
| Yarn characteristics:                                  |                |                |                |                 |                |                 |                |                 |
| reference elongation %                                 | 8.3            | 8.0            | 7.0            | 10.0            | 8.5            | 12              | 7.6            | 9.9             |
| break elongation %                                     | 18.4           | 19.0           | 17.8           | 22              | 19.8           | 24              | 13.5           | 16              |
| tenacity g/dtex                                        | 9.0            | 8.5            | 9.1            | 8.3             | 7.8            | 7.2             | 7.7            | 6.9             |
| Dry heat shrinkage %                                   | 7.9            | 7.8            | 8.2            | 8.0             | 3.5            | 3.7             | 3.5            | 3.6             |

We claim as our invention:

1. An improved process for the production of high-tenacity technical-grade yarns of polyamide and polyester, having a low reference elongation, by spin-drawing in which filaments extruded from a spinneret are cooled in a cooling zone by being exposed to a stream of air, said filaments being passed over a preparation device and then passed directly over a plurality of sets of rolls, said plurality of sets of rolls forming roll systems, said filaments being drawn between at least two sets of rolls in at least one draw field, said filaments being subjected to a temperature of greater than or equal to 160° C. on at least one set of rolls and subsequently being passed over a set of let-down rolls, constituting a let-down roll system, immediately prior to being wound up at a windup speed of greater than or equal to 2,200 m/min., the improvement comprising:

(a) heating a set of rolls, said set of rolls being positioned in advance of a minimum of one draw zone, said set of rolls being heated to a constant temperature, said temperature being in a range of ( $T_G - 20^\circ C.$ ) to ( $T_G + 65^\circ C.$ ), wherein  $T_G$  is the temperature of the glass transition point, said filaments being drawn over said set of rolls without the use of additional stationary draw means;

(b) maintaining a set of rolls at a temperature in excess of 110° C., said set of rolls being positioned following a minimum of one draw zone, said yarn having a tension of not less than 0.2 g/dtex upon leaving said roll system;

(c) permitting said yarn to remain in said let-down roll system for a residence time, said residence time being selected to be at least 0.2 sec.;

(d) maintaining said windup speed of said yarn at a speed not less than 2.5% less than the peripheral speed of said let-down roll system; and,

(e) adjusting the temperature of said let-down roll system to a temperature of less than or equal to 60° C.

2. The process of claim 1, wherein said filaments extruded from said spinneret are passed through a heated zone prior to entering said cooling zone.

20 3. The process of claim 1, wherein said filaments are prepared in said preparation device with an oil having less than 5% by weight of water, said oil being a water-deficient oil, said oil being applied to said filaments in the absence of heat.

25 4. The process of claim 1, wherein said let-down roll system is unheated and provided with cooling means, said cooling means providing a surface temperature of less than or equal to 25° C.

5. The process of claim 1, wherein said let-down rolls 30 are disposed in a cooling zone, said cooling zone having a temperature of less than or equal to 25° C. thereby enabling a heat exchange with said yarn.

6. The process of claim 5, wherein said yarn having a 35 residence time in said cooling zone, said residence time being adjusted to be at least 0.4 sec.

7. The process of claim 1, wherein said set of let-down rolls being positioned in a closed environment, said closed environment having a temperature, said temperature being maintained by forced cooling at or below 45° C.

40 8. The process of claim 1, wherein said yarn being withdrawn, said yarn having a tension of not less than 0.5 g/dtex.

9. The process of claim 1, wherein said set of rolls being positioned following a minimum of one draw zone, said set of rolls having a temperature of at least 160° C., said yarn leaving said set of rolls having a yarn tension of not less than 1.0 g/dtex.

50 10. The process of claim 1, wherein said yarn being of polyamide, said polyamide being polyamide-6, said yarn being characterized by a break elongation of less than or equal to 19% and a reference elongation of less than or equal to 8.5%.

11. The process of claim 1, wherein said yarn being of polyamide, said polyamide being polyamide-6, said yarn being characterized by a heat shrinkage of less than or equal to 4% and a reference elongation of less than or equal to 8.5%.

55 12. The process of claim 1, wherein said yarn being of polyester, said yarn being characterized by a heat shrinkage of less than or equal to 4% and a reference elongation of less than or equal to 9%.

\* \* \* \* \*